

United States Patent  
Dowling

[15] 3,685,449  
[45] Aug. 22, 1972

[54] EXPLOSIVE BOOSTER

[72] Inventor: Thomas P. Dowling, Whitehall, Pa.

[73] Assignee: Commercial Solvents Corporation

[22] Filed: Aug. 10, 1970

[21] Appl. No.: 62,676

[52] U.S. Cl.....102/24, 102/27

[51] Int. Cl.....F42b 3/10

[58] Field of Search.....102/24, 27

[56] References Cited

UNITED STATES PATENTS

2,733,658 2/1956 Moat .....102/24

3,037,453 6/1962 Cook et al. ....102/24  
3,212,438 10/1965 Lawrence.....102/24

Primary Examiner—Verlin R. Pendegrass  
Attorney—Howard E. Post and Robert H. Dewey

[57] ABSTRACT

An explosive booster for detonating insensitive blasting charges and a process for the manufacture thereof. The explosive booster has a core of detonating cord, the ends of which have been coated, encased in a sheath of relatively insensitive explosive material of high brisance.

3 Claims, No Drawings

**EXPLOSIVE BOOSTER****BACKGROUND OF THE INVENTION**

This invention relates to detonating means for relatively insensitive explosives and more particularly to boosters for insensitive explosives wherein reliable detonations are achieved through the use of a detonating cord core having the ends of said cord coated with a specific coating composition.

U.S. Pat. No. 3,359,902 to J. J. Minnick et al. and U.S. Pat. No. 3,037,453, incorporated herein by reference, describe explosive boosters having a core of detonating cord. Boosters of this type have been generally satisfactory in field use. However, some failures have been noted, especially when the boosters have been used under conditions wherein the boosters have been subjected to relatively high water pressures. The boosters of the present invention have been more reliable.

Accordingly, it is an object of the present invention to provide a new explosive booster.

It is another object of the present invention to provide a process for the manufacture of explosive boosters having high brisance and improved resistance to water.

These and other objects and advantages of the invention will be understood from the description of the invention.

**SUMMARY OF THE INVENTION**

The present invention provides an explosive device having a core of detonating cord substantially encased in a sheath of relatively insensitive explosive material. In the explosive device the terminals of the detonating cord are coated with a coating containing from about 60 percent to about 80 percent by weight of wax and from about 20 percent to about 40 percent by weight of polyethylene.

In the process of manufacturing such boosters, the terminals are coated with the coating composition at a temperature of from about 220° to about 240° F.

**DETAILED DESCRIPTION OF THE INVENTION**

Explosive boosters, having high brisance, for detonating relatively insensitive blasting charges, such as oiled ammonium nitrate, have been widely used and are generally very reliable. However, when explosive boosters having cores of detonating cord, generally of the type described in the U.S. Pat. Nos. 3,359,902 and 3,037,453, are used under conditions in which the booster is subjected to water pressure, some failures have been observed. Boosters are frequently subjected to relatively high water pressures when shooting "wet" holes.

Commercially available detonating cords, such as the widely used Primacord and E-cord, are substantially impervious to water. When loops of detonating cord are used as the explosive core in explosive boosters, the core is, therefore, also substantially impervious to water except that water can, of course, penetrate through the terminals. It was not believed that water penetration through the terminals of the detonating cord would be a problem because the cord was normally totally encased in a sheath of explosive material of high brisance which was itself substantially water im-

pervious. However, it has been discovered that during the manufacture of such explosive boosters that the terminals of the detonating cord frequently appear near or at the surface of the sheath of explosive material. Also, some of the explosive boosters have been found to have cracks in the sheath thereof. Any of such circumstances would, therefore, enable water to penetrate the detonating cord through the terminals thereof, and significant amounts of water in the detonating cord frequently inactivates the detonating cord causing failures of the explosive boosters.

It has now been discovered that the explosive boosters can be made significantly more reliable when the terminals are coated with a substantially waterproof coating composition. Specifically the coating composition contains from about 60 percent to about 80 percent by weight of wax and from about 20 percent to about 40 percent by weight of polyethylene. A coating composition of a substantially homogeneous mixture of 70 percent wax and 30 percent polyethylene is specifically preferred. Mixtures containing more than 80 percent wax are usually too thin to produce an acceptable seal and they do not give the desired water resistance. Mixtures containing less than 60 percent wax are generally too viscous to permit easy application of the coating and, further, they have a tendency to "block" readily. By "block" is meant that during manufacture adjacent coated terminals tend to stick together.

The wax used in the coating composition is preferably a paraffin wax. Other natural and synthetic waxes may, however, be used. The polyethylene, of course, has a melting point below 220° F. and specifically an emulsifier grade is used. Polyethylene used in coatings is commercially available from many sources. The wax and polyethylene are admixed into a substantially homogenous mixture at an elevated temperature before being applied to the terminals of the detonating cord.

The coating composition is applied to the terminals of the detonating cord in any suitable manner such as brush application, spraying, etc., although dipping of the ends into the coating composition is specifically preferred. The terminal is coated for at least one-fourth inch from the end and preferably at least one-half inch of the end of the detonating cord is coated. The coating composition is, of course, in molten form and preferably is at a temperature within the range of from about 220° F. to about 240° F. with a temperature of about 230° F. producing good results. Temperatures below 220° F. causes excessive "blocking" which results in large knobs of the coating composition at the end of the detonating cord. These knobs readily break off during handling, disturb the end seal thereby permitting the possible entrance of water into the detonating cord. Temperatures above 240° F. tend to cause the coating composition to attack the counteracting of the detonating cord, specifically the counteracting of reinforced Primacord, and result in a softening of the counteracting sealant and an unravelling of the counteracting fibers.

The following example, in the opinion of the inventor, represents the best embodiment of the invention.

## EXAMPLE

A mixture of 70 percent paraffin wax and 30 percent polyethylene having a melting point of 200° F. is heated to a temperature of 230° F. and mixed to obtain a homogeneous molten mixture.

Twelve 24 inch lengths of reinforced Primacord detonating cord had their terminals dipped to a depth of about 1 inch in the molten mixture to coat the ends and were then formed into bow-ties and used in the manufacture of explosive boosters as illustrated in the J. J. Minnick et al. U.S. Pat. No. 3,359,902. Torpex was used as the explosive sheathing material.

Explosive boosters were also made as above described in this example except that the terminals of the detonating cord were not coated.

Ten boosters having an explosive core of detonating cord of which the terminals were uncoated were subjected to water pressures of 80 p.s.i. for 16 hours and tested for sensitivity. When tested with a No. 6 cap in the cap well, four out of ten boosters failed to detonate.

Twelve boosters, having an explosive core of detonating cord of which the terminals were coated in accordance with the present invention, were subjected to water pressure of 80 p.s.i. for 16 hours and tested for sensitivity. When tested with a No. 1 cap in the cap

well, 11 out of the 12 detonated completely.

I claim:

1. In an explosive device having a core of detonating cord substantially encased in a sheath of relatively insensitive explosive material the improvement comprising a coating on the terminals of the detonating cord, said coating containing from about 60 percent to about 80 percent by weight of wax and from about 20 percent to about 40 percent by weight of polyethylene.
2. In a process for manufacturing an explosive device having a core of detonating cord substantially surrounded by a sheath of less sensitive explosive material, the steps comprising coating the terminals of the detonating cord with a sealing composition comprising from about 60 percent to about 80 percent by weight of wax and from about 20 percent to about 40 percent by weight of polyethylene, said coating being effected at a temperature of from about 220° to about 240° F., cooling the coating and subsequently surrounding the terminal-coated detonating cord with a sheath of explosive material less sensitive than said detonating cord.
3. The explosive device of claim 1 wherein said coating contains about 70 percent by weight of paraffin wax and 30 percent by weight of emulsifier grade polyethylene.

\* \* \* \* \*

30

35

40

45

50

55

60

65